

## UNITED STATES PATENT OFFICE

THOMAS THORNE BAKER, OF HATCH END, MIDDLESEX, ENGLAND, ASSIGNOR TO  
SPICERS LIMITED, OF LONDON, ENGLAND, A BRITISH COMPANY

## SOUND-RECORD CINEMATOGRAPH FILM

No Drawing. Application filed June 20, 1930, Serial No. 462,695, and in Great Britain July 1, 1929.

This invention comprises improvements in or relating to sound-record cinematograph films.

It is well known that, in the so-called talking films, the sounds are reproduced by means of a photographic record printed on a narrow strip about one-tenth of an inch in width at one side of the picture record. This invention relates to improvements whereby such 10 a strip would—in a colour film—be substantially an ordinary black and white photographic film devoid of any colour and allowing of the sound-record to be photographed in black and white.

15 Where the colours of the film depend upon a matrix or multicolor screen of primary colours over which the emulsion is coated, it is necessary to have an uncoloured transparent strip at one side of the cinematograph

20 film on which the sound-record is to be printed, for any pattern in a multicolor screen or matrix on the sound track (i. e. the portion of the film upon which the sound-record is printed) would give rise to high frequency

25 interruptions which would produce objectionable parasitic sounds or ground noise.

According to this invention in the manufacture of sound-record cinematograph films in natural colours, prior to the application of

30 the multicolor screen to the surface of the film, there is applied to that portion of the film which is to serve as the sound track, a layer of material to protect the underlying portion of the film from the dyes used in

35 making the multicolor screen.

In a preferred form of the invention the material employed to protect the sound track comprises a varnish such, for example, as bitumen dissolved in benzole.

40 A practical example of the method of carrying the invention into effect will now be given.

The film base, which comprises a cellulose acetate film, is coated along that portion which is to serve as the sound-track with a

45 strip of a bitumen-containing varnish of the necessary width (e. g. one-tenth inch). It is important that this layer of varnish should be only just sufficiently thick to prevent the layer of collodion which is next applied to the

50 film from attaching itself to that portion of

the surface of the film base which is protected by the strip of varnish. The varnish comprises a 1/2% solution of bitumen in benzole, and it is applied to the film by means of a small felt roller which is kept moist with the 55 varnish by means of a feeding roller.

A layer of collodion containing a green dye, the porosity of which layer has been increased by the addition thereto of 1 part in 4000 of water, is then applied to the whole 60 surface of the film. The multicolor screen is then formed on the surface of the collodion layer by ruling on lines of a fatty resist, bleaching the green dye from the spaces unprotected by the resist, re-dyeing the bleached 65 spaces in another colour and finally removing the resists in the manner described in U. S. Patent 1,805,361.

When the surface of the collodion layer is treated with benzole to remove the resists, 70 it will be found that the collodion is sufficiently porous to allow the benzole to penetrate through it and to dissolve the underlying bitumen. The strip of bitumen varnish, together with that portion of the collodion layer which overlies it, then comes away 75 from the film base, thus leaving bare a clear strip along the film base which serves as the sound track.

If desired, in order to obtain a three color 80 screen, a further strip of bitumen-containing varnish may be applied to the sound track, and a second series of lines of fatty resists can then be ruled on the film at an angle to the first series, and the bleaching, re-dyeing 85 and resist-removing operation can be repeated.

In the subsequent coating with sensitive emulsion there will thus be a strip of emulsion one-tenth of an inch in width with no 90 multicolor screen beneath it upon which the sound-record can be printed in the well-known manner.

I claim:—

1. A method of making a sensitive film of 95 the multicolor screen type for use in the production of sound record cinematograph films in natural colours which comprises applying to a cellulose acetate film, along a narrow strip which is to serve as a sound record 100

track, a layer of bitumen dissolved in benzole, coating the surface of the film with a layer of collodion, forming a multicolour screen on the collodion layer, treating the film with benzole to remove the bitumen together with that portion of the collodion layer which overlies the said layer of bitumen and finally coating the film thus prepared with a photographic emulsion.

10 2. A method of making a sensitive film of the multicolour screen type for use in the production of sound record cinematograph films in natural colours which comprises applying to a cellulose acetate film, along a narrow strip which is to serve as a sound record track, a layer of bitumen dissolved in benzole, coating the surface of the film with a layer of collodion containing a small proportion of water, forming a multicolour screen on the collodion layer, treating the film with benzole to remove the bitumen together with that portion of the collodion layer which overlies the said layer of bitumen and finally coating the film thus prepared with a photographic emulsion.

25 3. A method of making a sensitive film of the multicolour screen type for use in the production of sound record cinematograph films in natural colours which comprises applying to a cellulose acetate film along a narrow strip which is to serve as a sound record track, a layer of bitumen dissolved in benzole, coating the surface of the film with a layer of dyed collodion containing a small proportion of water, applying a series of lines of greasy ink to the collodion surface, bleaching the dye from the spaces unprotected by the lines of greasy ink, re-dying the bleached spaces in another colour, removing the lines 40 of greasy ink, treating the film with benzole to remove the bitumen together with that portion of the collodion layer which overlies the said layer of bitumen and finally coating the film thus prepared with a photographic emulsion.

45 4. A method of making a sensitive film of the multicolour screen type for use in the production of sound record cinematograph films in natural colours which comprises applying to a cinematograph film along a narrow strip which is to serve as a sound record track a layer of a resist material capable of protecting the underlying portion of the film from the action of dyes, coating the surface of the film with a layer of collodion porous to a solvent for the resist material, forming a multicolour screen on said collodion layer, treating the film with a solvent to remove the resist material, removing that portion of the 60 collodion layer which overlay the resist material, and finally coating the film thus prepared with a photographic emulsion.

55 5. A method of making a sensitive film of the multicolour screen type for use in the 65 production of sound record cinematograph

films in natural colours which comprises applying to a cinematograph film along a narrow strip which is to serve as a sound record track a protecting layer of bitumen dissolved in benzole, coating the surface of the 70 film with a layer of collodion porous to benzole, forming a multicolour screen on said collodion layer, treating the film with benzole to remove the bitumen together with that portion of the collodion lying thereover, and 75 coating the film with a photographic emulsion.

6. A method of making a sensitive film of the multicolour screen type for use in the production of sound record cinematograph 80 films in natural colours which comprises applying to a cinematograph film along a narrow strip which is to serve as a sound record track a layer of a resist material capable of protecting the underlying portion of the film 85 from the action of dyes, coating the surface of the film with a layer of collodion containing a small proportion of water, forming a multicolour screen on said collodion layer, treating the film with a solvent to remove the resist material, removing that portion of the 90 collodion layer which overlay the resist material, and finally coating the film thus prepared with a photographic emulsion.

In testimony whereof I affix my signature. 95  
THOMAS THORNE BAKER.

100

105

110

115

120

125

130